

1

3,087,774

## ANTIMICROBIAL COMPOSITION AND PROCESS FOR APPLYING SAME

Meyer Mendelsohn, New York, and Carl Horowitz, Brooklyn, N.Y., assignors, by mesne assignments, to Yardney International Corp., New York, N.Y., a corporation of New York  
No Drawing. Filed Oct. 12, 1959, Ser. No. 845,663  
12 Claims. (Cl. 8—115.5)

Our present invention relates to a treatment of fabrics and other materials with metallic compounds designed to impart antimicrobial properties to such materials.

In co-pending applications Ser. Nos. 738,967 and 760,857, filed by Meyer Mendelsohn on June 2, 1958, and September 15, 1958, respectively, both now abandoned, there has been disclosed a treatment of this character in which a zinc compound is caused to react on the fibers of a material to be treated, notably a cellulosic or proteinaceous material so that the zinc will firmly adhere to the fibers and exert its antimicrobial action even after repeated washings. More particularly, the treatment disclosed in these pending applications involves the immersion of the material in an aqueous bath at high temperatures, the bath including as its principal ingredients a chelating agent, a catalyst such as sodium acetate, and optionally a detergent along with a suitable zinc compound such as zinc chloride. A fixing agent rich in amine groups, such as urea, is applied to the material either in the same bath or in a second treatment solution to help lock the zinc in place on the fibers.

Although the treatment just described is satisfactory with respect to both the safety of operation and the quantity of zinc fixed in the fibers, there are nevertheless occasions when a more rapid mode of application is desirable. Thus, immersion of fabrics and the like for a prolonged period (e.g. 10 minutes) in a hot aqueous solution, followed by the necessary drying operation, represents a process which is practical only in industrial plants and can not be conveniently carried out in the home, in small institutions or in a store where an on-the-spot antimicrobial treatment of goods is desirable.

It is, therefore, an object of our present invention to provide an improved process for supplying such compositions to fibrous materials at ordinary temperatures and without the use of a slow-drying aqueous medium; a related object is to provide a modified antimicrobial composition adapted to be so applied.

In accordance with this invention we dissolve a zinc salt, a chelating agent, a catalyst, an aminating agent and preferably a detergent and buffering agent in an organic solvent, advantageously, a low-boiling ketone. When this mixture is applied, e.g. by spraying, to the material to be treated, it is found that the zinc compound reacts with the other ingredients to form a complex which remains fixed to the fiber over prolonged periods of use and exhibits distinct zones of inhibition against micro-organisms even after many washings in hot or cold water. It is further found that the use of low-boiling ketones is so effective in carrying the zinc into the fiber that a given percentage of zinc fixed in the fabric is obtainable with a greatly reduced proportion of zinc compound in the starting material, as compared with the hot-water treatment of the co-pending applications referred to above.

2

The following is a list of ketones found suitable for the process of our invention, the lower-boiling ones being preferred because of their shorter drying time.

TABLE 1  
Compound: Boiling point (° C.)

| Compound:                    | Boiling point (° C.) |
|------------------------------|----------------------|
| Trifluoro acetone            | 21                   |
| Acetone                      | 56                   |
| Hexafluoroacetyl acetone     | 63-65                |
| 2-butanone (ethyl methyl)    | 80                   |
| 3-buten 2-one (methyl vinyl) | 81                   |
| Biacetyl acetone             | 88                   |
| Methyl isopropyl ketone      | 94.3                 |
| Diethyl acetone              | 102                  |
| Methyl propyl ketone         | 102.3                |
| Pinacolone                   | 106                  |
| Methyl isobutyl ketone       | 116.8                |
| Cyclohexanone                | 156                  |

The following proportions (by weight) have been found to give a satisfactory mixture:

TABLE 2

| Zinc compound               | Parts    |
|-----------------------------|----------|
| 25 Aminating agent          | 5 to 300 |
| Chelating agent             | 1 to 100 |
| Catalyst                    | 1 to 350 |
| Detergent                   | 0 to 150 |
| Buffering agent             | 0 to 200 |
| 30 Volatile organic solvent | 1000     |

As an optional ingredient there may be added to the above mixture a commercially available moth-proofing agent soluble in the same solvent, such as from 1 to 50 parts of an alkali aluminum fluoride, or silico fluoride.

35 The zinc compound is preferably zinc chloride but may also be zinc sulphate or zinc nitrate.

### Example 1

40 A dry mixture is prepared as follows:

| Parts                                                                                                                           |
|---------------------------------------------------------------------------------------------------------------------------------|
| Anhydrous zinc chloride ZnCl <sub>2</sub>                                                                                       |
| Sodium acetate, 60% crystalline                                                                                                 |
| Boric acid (anhydrous)                                                                                                          |
| Anhydrous sodium ethylene diamine tetra acetate                                                                                 |
| 45 Detergent such as ethylene cycloimido 1-alkyl (fatty acid) 2-hydroxy ethylene sodium alcoholate methylene sodium carboxylate |

50 17.5 grams of the above mixture together with 17.5 grams of urea crystals are dissolved in 1000 grams of acetone. The resulting solution is sprayed at room temperature by means of an atomizer onto a piece of cotton or wool textile and allowed to dry for about two minutes.

55 A sample of the textile so treated is washed 20 times in a household washing machine with soap or detergent and is then placed on a Petri dish containing agar streaked with a culture of *Staphylococcus aureus*. After an incubation period of 24 hours a 2-mm. zone of inhibition is observed.

60 When the same mixture is sprayed on a piece of commercial air filter, a similar zone of inhibition is found to exist after 20 washings with a commercial detergent.

When a culture of *Escherichia Coli* is substituted for the *Staphylococcus aureus*, the zone of inhibition is found to be 3 mm.

65

## Example 2

The same as Example 1, except that cyclohexanone is used as a solvent in place of acetone. The solution dries in about five minutes.

A 1-mm. zone of inhibition against *Staphylococcus aureus* is observed after 20 washings.

## Example 3

Methyl isobutyl ketone is used as a solvent in lieu of those given in Examples 1 and 2. The drying time is about three minutes. The same zone of inhibition is observed as in Example 2.

It may be mentioned that the concentration of the mixture of the aforescribed solids in the organic solvent may vary from 0.1% to the saturation point, the latter being approximately 5%.

It should be noted that, especially with the addition of higher percentages of detergent or wetting agent, the composition according to the invention can also be used successfully on synthetic fibers, such as nylon.

Other alkali-metal acetates, such as potassium or lithium acetate, may be used as the catalyst in lieu of sodium acetate.

We claim:

1. An antimicrobial treating composition comprising a zinc salt, an aminating agent and a chelating agent all distributed in a volatile organic solvent.
2. A composition according to claim 1 wherein said volatile solvent is a ketone.
3. A composition according to claim 2 including as a catalyst an alkali-metal acetate.
4. A composition according to claim 3 including a detergent.
5. A composition according to claim 3 including a buffering agent.
6. As an article of manufacture, textile fiber impregnated with a composition comprising a zinc salt, an aminating agent and a chelating agent all distributed in a volatile organic solvent.

7. An article of manufacture according to claim 6 wherein the textile fiber is selected from the group consisting of cellulosic, proteinaceous and nylon fibers.

8. An antimicrobial treating composition comprising a zinc salt selected from the group consisting of zinc chloride, zinc sulfate and zinc nitrate; urea; sodium ethylenediamine-tetraacetate and a volatile organic solvent.

9. An antimicrobial treating composition according to claim 8 wherein said volatile organic solvent is a low-boiling ketone.

10. An antimicrobial treating composition according to claim 9 wherein said ketone is selected from the group consisting of acetone and methyl isobutyl ketone.

11. A process for imparting antimicrobial properties to textile fibers comprising applying to said fibers a solution of a zinc salt, an aminating agent and a chelating agent dissolved in a volatile organic solvent and allowing said solution to dry whereby antimicrobial properties are imparted to said textile fibers.

12. A process for imparting antimicrobial properties to textile fibers comprising applying to said fiber a solution of a zinc salt, a chelating agent dissolved in a volatile organic solvent, treating the fiber with an aminating agent and allowing said fiber to dry whereby antimicrobial properties are imparted to said textile fiber.

## References Cited in the file of this patent

## UNITED STATES PATENTS

|    |           |                |       |               |
|----|-----------|----------------|-------|---------------|
| 30 | 2,304,478 | Rosenzweig     | ----- | Dec. 8, 1942  |
|    | 2,396,514 | Kreidl et al.  | ----- | Mar. 12, 1946 |
|    | 2,459,896 | Schwarz        | ----- | Jan. 25, 1949 |
|    | 2,459,897 | Schwarz        | ----- | Jan. 25, 1949 |
|    | 2,525,049 | Signaigo       | ----- | Oct. 10, 1950 |
|    | 2,527,141 | Mantell et al. | ----- | Oct. 24, 1950 |
|    | 2,572,923 | Gaver et al.   | ----- | Oct. 30, 1951 |
|    | 2,609,368 | Gaver          | ----- | Sept. 2, 1952 |
|    | 2,671,779 | Gaver et al.   | ----- | Mar. 9, 1954  |
| 35 | 2,785,106 | Mendelsohn     | ----- | Mar. 12, 1957 |
| 40 | 3,004,010 | Mendelsohn     | ----- | Oct. 10, 1961 |